

May 30, 1939.

T. H. KRUEGER

2,159,993

LABEL AND LABELING

Filed June 18, 1936



INVENTOR  
*Theodore H. Krueger*  
BY *Edward Thomas*  
his ATTORNEY.

## UNITED STATES PATENT OFFICE

2,159,993

## LABEL AND LABELING

Theodore H. Krueger, Shelton, Conn.

Application June 18, 1936, Serial No. 85,943

7 Claims. (Cl. 216—62)

This invention relates to labels and labeling and is herein disclosed as embodied in a paper or textile label suitable for glass fruit jars and in a process of applying it.

5 Housewives have found the labeling of jars of preserves and jellies a laborious, exacting and messy job and have found the results uncertain,—the labels often peeled off by mere standing and those that did not peel off came off too easily 10 when moistened or stored in cellars. Moreover, it was necessary to apply paste to a label and apply the label to the jar, or to wet a previously glue-coated label, and, in either case, to apply the still wet label to the jar.

15 Among the other difficulties encountered were the need of allowing a hot, newly-filled jar of preserves to cool before applying the label, the impossibility of wiping the jar clean with a wet cloth after labeling without the probability of 20 loosening the label, and the annoyance of having a number of jars standing around while cooling and awaiting their turn to be labeled. Similar and other difficulties faced manufacturers who labeled vegetables and other products packed in 25 hot tin cans, and still other difficulties faced the user of labels on bottles and jars in a chemical laboratory.

According to the present invention these and other difficulties and objections are overcome, 30 and a label is provided which needs no moistening or application of paste but which, though normally non-sticky, becomes adhesive upon being placed against the hot jar or other heat-conducting container, and adheres thereto, the adhesive being softened by the heat so as to cause 35 the label to adhere but not become so liquid or so bulky as to permit the label to slip along the jar by its own weight.

Thus the heat of the jar is the element which 40 causes the normally non-adhesive label to become adhesive and adhere to the jar.

Other features and advantages will hereinafter appear.

In the accompanying drawing a jar 1, having 45 a top 2 contains hot preserves.

On the hot cylindrical side of the jar has been laid a label 3 having a coating diagrammatically shown at 4 on its back in which causes it to adhere to the glass.

50 Not every heat-softened coating 4 is satisfactory for the coating must remain hard, or hard enough to resist slipping, up to temperature of about 120° F. and usually must soften to an adhesive at a temperature well below the boiling point of water, and below that at which the cellu-

lose body scorches, that is it must serve as an adhesive at a temperature at least as low as 180° F. It must also stick to glass if used on glass jars.

The most satisfactory adhesive yet found is the homogeneous substance obtained when paraffine wax of 130° to 132° F. melting point is heated and 5 6% to 30% of thin R. C. M. A. crepe rubber is dissolved in it at 200° F. in sheets not exceeding .004 inch thick, and the resulting mass is kneaded in a Werner Pfleiderer class III type BB mixer 10 and mixed until homogeneous.

It is possible to substitute gutta percha for the rubber. Some synthetic resins and some compositions containing nitro-cellulose and plasticizer may also be substituted for the adhesive de- 15 scribed, but such are generally more expensive and seemed less satisfactory to work with. One such is nitro-cellulose combined with glyptyl or rezyl resins dissolved in a solvent with a plasticizer, the resin being compatible with the cellulose. 20 Other wax, such as ceresine, may replace paraffine.

The heat-softened coating described is adapted to be softened a second time to reset the label.

Usually one edge of the label is applied to the 25 hot jar to center the label and then the whole label is smoothed down.

If desired the label may be applied to a cold body by rubbing it on to the body by a hot rubbing surface.

Having thus described certain embodiments of the invention in some detail, what is claimed is:

1. A label having a body and a heat-softenable back of normally non-sticky composition dependent upon the presence of paraffine wax and rubber to become adhesive when heated.

2. A paper label carrying on its back a normally non-sticky composition of paraffine wax and rubber, and adapted to adhere to glass when heated.

3. A label having a cellulose body and a heat-softenable normally non-sticky back adapted to become adhesive and cling to a jar when heated to an elevated temperature not exceeding 180° F.

4. The process of labeling hot heat-conducting containers which consists in applying to the hot container a label bearing on its back a normally non-sticky heat-softenable adhesive becoming adhesive when heated at an elevated temperature between 120° and 180° F.

5. The process of labeling hot jars which consists in applying to the hot jar a label bearing on its back a normally non-sticky heat-softenable adhesive becoming adhesive when heated at an elevated temperature between 120° and 180° F.

6. The process of labeling hot heat-conducting containers which consists in applying to the hot container a label having a heat-softenable back of normally non-sticky composition dependent upon the presence of wax and rubber to become adhesive when heated at a temperature between 120° and 180° F.

7. The process of labeling hot heat-conducting containers which consists in applying to the hot container a label carrying on its back a normally non-sticky composition of paraffine wax and rubber, which becomes adhesive when heated at a temperature between 120° and 180° F.

THEODORE H. KRUEGER.